

June 6, 1967

J. A. NELSON ET AL

3,323,881

FERROUS BASE COATED WITH ZINC AND CHROMIUM

Filed Nov. 29, 1963



Inventors

John A. Nelson

Fred E. Wills

By Hibben, Noyes & Bicknell

Attorneys

## 1

3,323,881

FERROUS BASE COATED WITH ZINC  
AND CHROMIUMJohn A. Nelson, Tucson, Ariz., and Fred E. Wills, Gary,  
Ind., assignors to Inland Steel Company, Chicago, Ill.,  
a corporation of DelawareFiled Nov. 29, 1963, Ser. No. 326,809  
6 Claims. (Cl. 29—183.5)

The present invention relates generally to the production of a ferrous metal sheet and strip material having a protective metal coating thereon, and more particularly to a galvanized steel sheet or strip material having improved resistance to corrosion.

The increased competition offered to galvanized steel sheet and strip products by other materials of construction makes it increasingly desirable to provide galvanized steel sheet and strip products having improved resistance to corrosion which can be produced at a cost competitive with other materials of construction, such as aluminum or plastic coated sheet materials. And, since an appreciable quantity of galvanized strip and sheet material is used by forming or drawing, it is highly desirable that the galvanized sheet and strip material be capable of being formed or drawn without adversely affecting the corrosion resistance thereof.

It is therefore an object of the present invention to provide ferrous metal strip and sheet products having improved corrosion resistance.

It is also an object of the present invention to provide a ferrous metal strip having improved corrosion resistance by treating a ferrous metal strip in-line with a continuous metal coating line.

It is a further object of the present invention to provide markedly improved corrosion resistant galvanized steel strip and sheet products which can be produced continuously in-line with a continuous galvanizing process line.

It is another object of the present invention to provide galvanized steel strip and sheet materials which have imparted thereto markedly improved corrosion resistance without having the general utility of the galvanized materials impaired.

It is still another object of the present invention to provide galvanized steel strip and sheet products having greatly improved corrosion resistance which are capable of being drawn or formed without impairing the corrosion resistance thereof.

Other objects of the present invention will be apparent from the following detailed description when read in conjunction with the accompanying drawing and claims to follow.

Heretofore it has been thought that very thin chromium coatings applied directly over zinc on a steel base would have no beneficial effect, since very thin coatings of chromium were not thought capable of adhering to a galvanized surface and forming an impervious coating directly thereover. It has also been found that very thin chromium films having a thickness of .00002 inch when applied directly on the ferrous metal surface of a steel strip do not improve the salt spray corrosion resistance of the steel strip.

It has now been discovered, however, that the corrosion resistance of a galvanized conventional low carbon steel strip or sheet, such as produced on a continuous hot dip or electrolytic galvanizing line, can be greatly improved with regards to its corrosion resistance by applying continuously to the as plated or temper rolled zinc coating as it leaves the continuous galvanizing line a very thin film of electrolytically deposited chromium having a thickness range from at least about .000001 inch but less than

## 2

.00002 inch with a preferred thickness being from about .000004 inch to about .00001 inch. An extremely thin chromium coating having the foregoing thickness range can be readily applied to a galvanized steel strip electrolytically within the time and space limitations imposed by a conventional in-line continuous galvanizing process line as the strip leaves the galvanizing line and while traveling at its normal rate. Thus, it is possible for the first time to produce a galvanized steel strip or sheet product having very substantially improved corrosion resistance in a more economical manner than heretofore. And, because the chromium film is extremely thin, the chromium coated galvanized steel strip or sheet can be formed or drawn in the same manner as the uncoated galvanized strip or sheet without destroying the improved corrosion resistance which has been imparted thereto.

More particularly, in accordance with the present invention, a galvanized steel strip of any conventional type, such as a low carbon steel strip having a thin coating of zinc thereon, preferably between about .0001 inch to .002 inch in thickness, exhibits substantially improved corrosion resistance when a thin film of chromium having a thickness of as little as .000001 inch is electrolytically deposited directly on the surface of the zinc coating. In the accompanying drawing, the graph showing the relationship between the electrolytically applied chromium film thickness and the corrosion ratio<sup>1</sup> of a chromium coated conventionally hot dip galvanized steel strip having on each side thereof a zinc coating thickness of about .0005 inch indicates that there is a very substantial increase in the corrosion resistance of a galvanized steel strip when a film of chromium having a thickness of only .000001 inch is provided directly on the galvanized surface and that the corrosion resistance continues to increase at a fairly rapid rate as the thickness of the chromium film is increased to about .000004 inch. There does not appear to be any increase in corrosion resistance of the galvanized strip as the continuously electroplated chromium film is increased in thickness above .00001 inch to about .00002 inch. The failure to obtain any increase in corrosion resistance with the thicker chromium film may be due to the formation of cracks therein. Actually, increasing the coating thickness of the chromium film from .000004 inch to .00001 inch only increases the corrosion ratio from about 1.9 to 2.0, and this slight increase amounting to 5% is obtained by a 2.5-fold increase in the chromium coating thickness. From a commercial viewpoint it would appear inadvisable and unnecessary to employ a chromium coating having a thickness in excess of about .00001 inch and probably not above .000004 or .000005 inch.

The improvement in corrosion resistance is effected by applying an extremely thin film of chromium of the herein disclosed type to any of the conventional galvanized steel sheet or strip materials, including both conventional hot dip galvanizing and electrolytic galvanizing steel sheet and strip materials. In the following Table I are shown the test results achieved by chromium plating in accordance with the present invention two conventional steel mill produced hot dip galvanized steel products of the indicated types:

<sup>1</sup> The "corrosion ratio" value =

Time to failure of sample  
Avg. time to failure of controls

The failure of a sample or control is indicated by the first appearance of red rust thereon. If the corrosion ratio value is greater than 1.0, the resistance to corrosion is improved; if less than 1.0, the corrosion resistance is impaired. A corrosion ratio of 2.0, for example, indicates an increase in corrosion resistance of 100% over the control.

TABLE I.—EFFECT OF CHROMIUM PLATING ON THE 5% SALT SPRAY TEST PERFORMANCES OF MILL PRODUCED GALVANIZED STEELS

| Type of Galvanized Steel Products | Corrosion Ratios            |                             |                             |                            |
|-----------------------------------|-----------------------------|-----------------------------|-----------------------------|----------------------------|
|                                   | Chromium Coating, .0015 mil | Chromium Coating, .0025 mil | Chromium Coating, .0035 mil | Chromium Coating, .005 mil |
| Extra Smooth-----                 | 1.4                         |                             | 1.7                         | 2.0                        |
| Minimum Spangle-----              | 1.5                         | 1.7                         |                             | 2.0                        |

It will be evident from Table I that the corrosion resistance of conventional galvanized sheet material of the type normally produced on a standard continuous galvanizing line and having the specified thin chromium film applied directly over a standard zinc spelter hot dip coating is not affected by the temper rolling of the galvanized strip before chromium plating, since the corrosion ratios of the respective temper rolled (i.e. extra smooth) materials were of the same general magnitude as when not temper rolled before chromium plating. These chromium coated strips can be drawn and formed without destroying their improved corrosion resistance.

In the following Table II are shown the results achieved when hot dip galvanized sheet material and electrogalvanized sheet materials of the specified type are subjected to a standard continuous 5% salt spray test for corrosion resistance after coating with a thin film of chromium in accordance with the present invention:

TABLE II.—EFFECT OF CHROMIUM COATING ON THE 5% SALT SPRAY TEST PERFORMANCES OF VARIOUS TYPES OF GALVANIZED STEEL SHEETS

A—HOT DIP GALVANIZED COATING<sup>1</sup>

| Zn Coating Weight/Side | Chromium Coating, Thickness | Corrosion, Ratio | Number Hours to Red Rust |
|------------------------|-----------------------------|------------------|--------------------------|
| .50 oz./sq. ft-----    | (None)-----                 | Control          | 800                      |
| .50 oz./sq. ft-----    | .002 mil-----               | 2.3              | 2,000                    |
| .40 oz./sq. ft-----    | (None)-----                 | Control          | 600                      |
| .40 oz./sq. ft-----    | .002 mil-----               | 2.0              | 1,200                    |

B—ELECTRO GALVANIZED COATING<sup>2</sup>

| Zn Coating Weight/Side | Chromium Coating, Thickness | Corrosion, Ratio | Number Hours to Red Rust |
|------------------------|-----------------------------|------------------|--------------------------|
| .25 oz./sq. ft-----    | .005 mil-----               | 4.2              | 1,310                    |
| .25 oz./sq. ft-----    | .007 mil-----               | 4.3              | 1,371                    |
| .25 oz./sq. ft-----    | (None)-----                 | Control          | 312                      |

<sup>1</sup> Zn Coating comprised a .05% Mg., Lead-free Zinc Spelter.

<sup>2</sup> Plated from Standard Electrolytic Zinc Plating Bath.

It is evident from Table II that an extremely thin chromium surface film substantially increases the corrosion resistance of the hot dip galvanized and electrolytic zinc coated steel materials. The salt spray test performances of these chromium plated strips hot dip coated with the special lead-free zinc spelter containing .05% magnesium having a zinc coating weight of only .40 ounce per ft.<sup>2</sup> and a chromium film thickness of only .000002 inch (.002 mil) ranged from about 1200 to 2000 hours, and these are approximately four to six times better than that of regular hot dip galvanized steel strips having a heavier zinc coating weight but without the extremely thin chromium surface film.

In the tests of the electrogalvanized chromium coated samples reported in Table II, the corrosion ratios obtained were extremely high, approximately 4.2, for a chromium coating thickness of .000005 inch to .000007 inch. This is twice as high as has been obtained with similarly chromium coated hot dip galvanized steel samples. Moreover, an electrolytic zinc coating weight of only .25 oz. per square foot per side was used to obtain these very high corrosion ratios. Thus, even with very thin electrolytically applied zinc coatings, applying a chromium film increases the corrosion ratio of the electrogalvanized strip about four times.

The thin chromium surface films employed in the present invention can be applied electrolytically by any conventional chromium plating procedure and by any conventional chromium plating bath to produce a bright chromium surface film. The composition of several aqueous plating baths, including special high speed plating solutions, and the operating conditions which can be employed are shown in the following Table III:

TABLE III.—PLATING CONDITIONS FOR VARIOUS CHROMIUM PLATING BATHS

| Type of Cr Plating Bath |                                                                                                  | Bath Temp., °F. | Current Density—Amperes |
|-------------------------|--------------------------------------------------------------------------------------------------|-----------------|-------------------------|
| Normal-----             | Chromic Acid 250 g/l., Sulfuric Acid 2.55 g/l.                                                   | 130             | 120/sq. ft.             |
| Bornhauser-----         | Chromic Acid 297 g/l., Caustic Soda 57.7 g/l., Trivalent Chrom. 7.5 g/l., Sulfuric Acid—0.7 g/l. | 65              | 300/sq. ft.             |
| Unimet CR 110*-----     | Chromic Acid 225 g/l., Sulfuric Acid 5 g/l., Addition Agents.                                    | 130             | 340/ft. <sup>2</sup>    |
| Unimet CF 520*-----     | Chromic Acid 370 g/l., Sulfuric Acid 2.25 g/l., Addition agents.                                 | 120             | 240/ft. <sup>2</sup>    |

\*Produced by Metal Thermit Corporation.

In the following Table IV there is shown a comparison of the corrosion resistance of a conventional hot dip galvanized steel strip product having a uniform coating weight of about .603 oz./ft.<sup>2</sup> per side (i.e. coating thickness per side of about .0005 inch) coated by one of the above indicated chromium plating baths under the conditions specified:

TABLE IV.—COMPARISON OF VARIOUS CHROMIUM PLATING BATHS—  
5% SALT FOG TEST RESULTS

| Chromium Plating Bath | Time, Sec. | Current Density, Amps per ft. <sup>2</sup> | Temp., °F. | Plating Thickness, mils | Samples Failure, Hours to Red Rust | Corro-<br>sion Ratio |
|-----------------------|------------|--------------------------------------------|------------|-------------------------|------------------------------------|----------------------|
| Normal                | 10         | 120                                        | 130        | .001                    | 672                                | 1.72                 |
|                       | 10         | 120                                        | 130        | .001                    | 648                                | 1.66                 |
|                       | 60         | 120                                        | 130        | .005                    | 696                                | 1.78                 |
|                       | 60         | 120                                        | 130        | .005                    | 816                                | 2.10                 |
| Bornhauser            | 10         | 300                                        | 65         | .001                    | 480                                | 1.23                 |
|                       | 10         | 300                                        | 65         | .002                    | 792                                | 2.02                 |
|                       | 60         | 300                                        | 65         | .003                    | 696                                | 1.78                 |
|                       | 60         | 300                                        | 65         | .004                    | 840                                | 2.15                 |
| Unimet CR 110*        | 10         | 340                                        | 130        | .004                    | 480                                | 1.23                 |
|                       | 10         | 340                                        | 130        | .004                    | 576                                | 1.47                 |
|                       | 60         | 340                                        | 130        | .020                    | 672                                | 1.72                 |
|                       | 60         | 340                                        | 130        | .020                    | 696                                | 1.78                 |
| Unimet CF 520*        | 10         | 240                                        | 120        | .003                    | 792                                | 2.02                 |
|                       | 10         | 240                                        | 120        | .003                    | 648                                | 1.66                 |
|                       | 60         | 240                                        | 120        | .010                    | 840                                | 2.15                 |
|                       | 60         | 240                                        | 120        | .020                    | 746                                | 1.91                 |

\* Produced by Metal Thermit Corporation.

Since there is no marked advantage resulting from using any of the special chromium plating baths, it is preferred to apply the thin chromium film by means of a normal chromium plating both of the type disclosed in Table III, particularly since the latter is more easily controlled than any of the other chromium plating baths which have been tested.

In applying the extremely thin chromium film to the surface of a zinc coating on a steel strip the usual good operating practice should be followed and the zinc surface when chromium plated should be free of surface oxides and contamination. A bright chromium surface film can be plated from a normal chromium acid sulfate plating bath without benefit of any special pre-treatment when a clean oxide-free zinc surface is presented. If desired, however, a standard bright dip can be applied to the zinc coated strip immediately before electroplating. An electrolytic pre-treatment which results in forming an oxide film on the zinc coating should be avoided where a bright appearing final product is necessary. If desired, the resultant chromium plated galvanized steel strip can be further treated to provide satisfactory wet storage stain resistance without impairing its corrosion resistance by subjecting the plated strip to a conventional chromate treatment, such as a three second treatment in about a .3% ammonium chromate solution.

As previously indicated, the present invention can be readily incorporated into a conventional continuous galvanizing line, since the extremely thin chromium film required in the present invention can be electrolytically applied by means of conventional electroplating equipment within a matter of seconds and therefore does not require extensive space which would make the chromium plating treatment entirely impractical for continuous in-line processing with a continuous galvanizing line. For example, a commercial continuous galvanizing line treating a 48-inch wide low carbon steel strip normally runs at a rate of 100 ft./min. for 20 gauge steel strip material, and at a rate of 150 ft./min. for 24 gauge material when operating under normal conditions. If we assume that a galvanizing line is producing 48-inch width material having a 24 gauge thickness and traveling at a rate of 150 ft./min., the amperage required to apply a .00001 inch chromium coating on both sides at a current efficiency of 20%, is about 200,000 amperes. The plating

section is preferably a horizontal multi-tiered unit in which one side of the galvanized strip is plated in one tier and the other side is plated in the second tier. At the present time the maximum current that can be transferred to a strip is equivalent to a current density of 300 amperes per square foot. Under the foregoing conditions, the length of the plating section is approximately

85 feet. This length of plating section gives a plating time for the above product of approximately 33 seconds. If a chromium film having a thickness at the lower end of the preferred range of chromium coating thickness is used, the length of the foregoing plating section is reduced to approximately 43 feet when chromium plating under the same operating conditions. It should also be understood that, while possible, it is considerably more expensive to provide a chromium film on the galvanized steel strips or galvanized cut sheet material in accordance with the present invention after the continuous strip has been removed from the continuous galvanizing line and furthermore introduces additional operating problems which are entirely avoided by the preferred in-line treatment.

In the foregoing description, data and examples illustrating the present invention wherein zinc coatings are referred to and used, it should be understood that the "zinc coating" can be composed of zinc or any conventional or special zinc alloy formulation. And, whereas the specific embodiments of the present invention have used zinc for the protective metal coating on the ferrous metal strip base material, other protective metals, such as cadmium, aluminum, or alloys thereof, can be used in place of zinc and come within the broad scope of the present invention.

We claim:

1. A ferrous metal product comprising a ferrous metal strip with a protective metal coating containing zinc on at least one surface thereof with said coating having electrolytically applied directly thereon a thin surface film of metallic chromium having a substantially uniform thickness ranging between at least about .000001 inch and less than .00002 inch, whereby said galvanized steel product is provided with a substantially improved corrosion resistance.
2. A steel product as in claim 1, wherein said zinc coating has a thickness of about .0001 inch to .002 inch.
3. A steel product as in claim 1, wherein said zinc coating is a hot dip galvanized zinc coating consisting essentially of a lead-free zinc spelter containing about .05% magnesium.
4. A steel product as in claim 1, wherein said zinc coating is an electrolytically deposited layer of zinc.

5. A steel product as in claim 4 wherein said zinc coating has a thickness of about .25 oz./sq. ft. of surface area.

6. A steel product having a protective metal coating comprised essentially of zinc exhibiting substantially improved corrosion resistance and good drawing properties which comprises; a steel strip having a protective metal coating comprised essentially of zinc on at least one surface of said strip, and said protective coating having a film of metallic chromium electrolytically applied directly on said coating with said film having a substantially uniform thickness between about .000004 inch and .00001 inch.

## References Cited

## UNITED STATES PATENTS

|           |         |               |       |            |
|-----------|---------|---------------|-------|------------|
| 1,615,585 | 1/1927  | Humphries     | ----- | 29—196.6   |
| 1,663,215 | 3/1928  | Peirce et al. | ----- | 75—178     |
| 1,998,496 | 4/1935  | Fiedler.      |       |            |
| 2,294,750 | 9/1942  | Harris.       |       |            |
| 2,658,266 | 11/1953 | Du Rose       | ----- | 29—196.6 X |
| 2,918,722 | 12/1959 | Kenmore       | ----- | 204—55     |
| 3,063,918 | 11/1962 | Kennedy       | ----- | 29—65      |
| 3,106,484 | 10/1963 | Miller        | ----- | 209—41 X   |

HYLAND BIZOT, Primary Examiner.